

1,318,891.

J. R. MACMILLAN,  
MANUFACTURE OF MANGANATES,  
APPLICATION FILED JUNE 11, 1918.

Patented Oct. 14, 1919.

2 SHEETS—SHEET 1.

*Fig. 1.*



### Inventor

J. R. MacMillan

K.P. McElroy  
Attorney

WITNESS:

WITNESS:-  
Chas. L. Grossblauer  
Hilda Schoenthal.

1,318,891.

J. R. MACMILLAN.  
MANUFACTURE OF MANGANATES.  
APPLICATION FILED JUNE 11, 1918.

Patented Oct. 14, 1919.

2 SHEETS—SHEET 2.

Fig. 2.



Fig. 3.



### Inventor

J.R. MacMillan

**WITNESS:-**

WITNESS:-  
Chas. L. Griesbauer  
Hilda Schonenthal.

ପତ୍ର

K.P. McElroy  
Attorney

# UNITED STATES PATENT OFFICE.

JOHN R. MACMILLAN, OF NIAGARA FALLS, NEW YORK.

## MANUFACTURE OF MANGANATES.

1,318,891.

Specification of Letters Patent. Patented Oct. 14, 1919.

Application filed June 11, 1918. Serial No. 239,493.

To all whom it may concern:

Be it known that I, JOHN R. MACMILLAN, a citizen of the United States, residing at Niagara Falls, in the county of Niagara and

5 State of New York, have invented certain new and useful Improvements in the Manufacture of Manganates, of which the following is a specification.

This invention relates to the manufacture 10 of manganates; and it comprises a method of making alkaline manganates, such as sodium manganate, wherein a mixture of manganese oxid and caustic alkali is submitted to a grinding or comminuting operation at 15 a temperature sufficient to cause free absorption of atmospheric oxygen; all as more fully hereinafter set forth and as claimed.

In the manufacture of permanganates and manganates, it has long been the practice to 20 heat a mixture of manganese dioxide,  $MnO_2$ , with a caustic alkali, usually caustic soda or caustic potash, in the presence of air or oxidizing materials. Barytes, lime, etc., are more rarely used. By a well understood reaction, under these conditions some or all of 25 the manganese dioxide takes up an additional atom of oxygen and unites with the alkali to form a manganate, such as  $Na_2MnO_4$ . From this manganate a permanganate is afterward 30 made by methods not here important. In principle the reaction is simple; but it is one difficult to carry out on any large commercial scale, this being partly because of the corrosive and caustic properties of the 35 alkali and partly because of the physical character of a mixture of readily fusible alkali and infusible manganese dioxide (per-oxid). If air be relied on to furnish the necessary oxygen, absorption is slow at low 40 temperatures and at higher the mixture becomes a pasty mass hard to handle. For any quick action, air must of course have free access to every portion of the mass and this is difficult to secure. With aerial oxidation, the mixture is usually heated in a 45 reverberatory furnace with free access of air above the hearth and is rabbled or stirred by workmen; a matter of some difficulty for the noted reasons. As usually conducted, 50 complete oxidation of the mass requires a long time and much labor if any substantial quantity is being handled. In practice, in order to make the work easier, it is customary to use an excess of caustic soda over that

theoretically required; this excess making 55 the mass somewhat thinner and easier to work and also accelerating the formation of manganate.

I have found that I can effect a rapid and complete oxidation of manganese dioxide to 60 form sodium manganate by air at a relatively low temperature, say 400° to 550° C., by simply grinding or comminuting the mass of the mixture of dioxide and caustic soda in a hot mill in such a manner as to expose 65 extensive and constantly changing faces to the action of air. In so doing every particle of the dioxide in the mass is positively exposed to action of the air and the attack of the air and alkali on it is much hastened. 70 In effect, I secure a quick action at a low temperature; a temperature at which the mechanical properties of the mass are not so inconvenient as in prior methods. It may be, indeed, with proper proportioning of 75 materials a readily disintegrating or "dry" mass breaking down into a powdery consistency. The grinding or comminution sought is that of the mass as a whole; not that of the manganese dioxide since I ordinarily preliminarily grind this as fine as practicable. Any convenient type of mill set in or on a suitable heating furnace and provided with 80 means for causing passage of air in proximity to the grinding surfaces may be employed; but I find that it is best to use a mill of the type of a "chaser mill"; a mill in which one grinding surface is afforded by a bottom plate or element over which another grinding element travels. Such a mill 85 may be simply set on a furnace chamber with its bottom plate forming the furnace top; or the grinding elements may be electrically heated. Any means of securing the necessary temperature at the point of grinding 90 may be used. It is best to inclose the mill in a suitable housing to keep in dust. In practice, using suitable apparatus, I find that I can secure a substantially complete 95 oxidation of a charge in from ten minutes to an hour. The mill may or may not be continuously operating.

In a practical embodiment of the present invention, I first make a mixture of commercial fine ground manganese binoxid, or other suitable form of manganese oxid, with ordinary commercial caustic soda, flaked or ground, heat the mixture to drive off water 105

and dry it and transfer to a hot mill for grinding and oxidation. If potassium manganate and permanganate are desired, the equivalent quantity of caustic potash may be substituted. One good mixture for the present purposes consists of 50 parts of commercial fine ground natural manganese bin-  
 5 oxid or peroxid and 75 to 100 parts of ordinary dry commercial caustic soda. Ore of a  
 10 fineness of 150 to 200 mesh is well suited for the present purpose. With the proportions stated, the caustic soda is in excess of the theoretical requirements and the mixture is moreover rather too pasty when hot for convenient work. The excess of soda however quickens oxidation. Ordinarily I find it better to use about the theoretical amounts, as in using a mixture of about equal parts  
 15 of a good grade of manganese ore and caustic soda. Recovered manganese oxids may be used instead of the natural minerals. A good mixture is 100 parts of recovered oxid and 75 parts of caustic soda. As stated, in lieu of caustic soda, the equivalent amount of  
 20 caustic potash may be substituted. Whatever the proportions of manganese oxid and alkali, the mixture is usually put on a plate, which may be of iron, and is heated by fire heat underneath until it dries out and becomes hot and powdery. This preliminary heating usually results in a certain amount  
 25 of oxidation, thereby lessening, concomitantly, the time necessary in the next operation. The hot dry mixture is next hot-  
 30 ground until a substantially complete conversion is obtained, this requiring a time which varies with the character of the mixture, the temperature and the grinding mill. Ordinarily I use a temperature between 400°  
 35 and 550° during the comminution and oxidation; this temperature being that of the mass under treatment. It is not necessary that the whole apparatus be at this temperature; or that the temperature be uniform through-  
 40 out. Through the mill casing air is slowly drawn or passed in such a manner as to insure a sufficient supply at the grinding surfaces. If the mill is of a continuously operating type, feed of raw mixture and dis-  
 45 charge of finished manganate may be continuous; but otherwise I charge the mill and slowly grind the mixture until oxidation has gone as far as may be desired. The charge is then removed and cooled and treated in  
 50 the usual manner to make commercial manganate or permanganate as the case may be.

The operation is exactly the same in making potassium manganate, barium manganate, strontium manganate, calcium manganate, etc., the corresponding alkali being simply substituted in equivalent amounts for the caustic soda in the examples given. Carbonates may be substituted for caustic alkali.

In the accompanying illustration I have  
 65 shown, more or less diagrammatically, cer-

tain apparatus within this invention and useful in the performance of the described process. In this showing

Figure 1 is a side elevation;

Fig. 2 is a top plan view, and

Fig. 3 is an elevation taken at the right of Fig. 1.

In the drawings, the furnace consists of two heating chambers, 1 and 2, each provided with tiers of refractory material 3, 75 advantageously in brick-like form, serving to direct the heat and flames toward the top of the chambers. Stack 4 in communication with chamber 1 serves to produce the necessary draft and remove the waste gases. The 80 furnace chambers may be fired by means of oil burners (not shown) or other firing means of any usual construction. A mixture of a suitable manganese oxid and caustic alkali is preheated or dried on the plate 5 over 85 heating chamber 1 and is delivered thence into a chaser mill mounted over chamber 2. The mill as shown comprises standards 6 and 7 having a shaft 8 journaled therein with pulley wheel 9 keyed to the shaft. 90 Driving pinion 10 attached to the shaft serves to drive the beveled gear 11 which in turn is keyed to shaft 12 having a bearing at 13 supported by a cross beam 14 connecting the two standards. Shaft 12 operates an 95 enlarged extension 15 seated in the bearing 16 on the plate 17. This plate forms one of the grinding elements and is mounted over the top of the chamber 2. This extension 15 is bored at 18 to receive the horizontal shaft 100 19 carrying at either end roller elements 20 adapted to bear directly upon the plate 17. It may also carry stirring elements shown as chains 20' pivoted thereto, for turning and stirring the mass and pushing it into the 105 path of the grinding rolls. Above this plate are upwardly extending walls 21 to confine the material. The rollers 20 may be adjusted with respect to the grinding plate by means of the nut 22 on shaft 12. The mill 110 is advantageously inclosed by a hood 23, which has an opening 24 at one side in proximity to plate 5 of the heating chamber 1. This opening serves for the introduction of the predried mixture and for supplying air. 115 In communication with the hood is a flue 25 leading to an exhaust fan 26. The amount of air passed over the material may be regulated by regulating the speed of this fan. Any dust resulting from the grinding operation goes forward to the exhaust means and may be recovered by any suitable means (not shown). Exit gases are sent away to waste or to a place of disposition through exhaust flue 27. The fan is mounted above 125 the mill upon a standard or support which advantageously is as shown an I-beam 28 carrying bracket 29 supporting the fan. Pulley 30 mounted on shaft 31 in bracket 32 serves for driving the fan.

The operation of the apparatus is clear from the foregoing. The material is pre-dried upon the plate 5, shoveled through opening 24 on plate grinder 17 over the 5 heating chamber 2 where it is subjected to comminution and aeration. The roller elements, in addition to comminution, perform an effective rabbelling. To remove the charge of finished manganates, hood 23 may be detached or the material may be removed 10 through door 24. With the proper proportions and temperatures, no inconvenient sintering or fusion occurs, the mass remaining "dry" and easily ground throughout and 15 the finished material is delivered as a powdery product, readily handled. It is not necessary to increase the amount of manganese binoxid above the amount necessary for conversion into manganate with the soda 20 present, in order to secure a dry readily handled composition; although this may be done.

I regard as within my invention any process of mixing alkali and a manganese oxid 25 and hot grinding the mixture at a temperature where it will remain substantially dry but nevertheless will absorb atmospheric oxygen freely. Oxidants may be incorporated in the mass but their use is not necessary. Where an excess of manganese binoxid is used this may function to give oxygen according to a well understood reaction. I find that for the present purposes a temperature of 400° to 550° C. at the grinding 30 surfaces is desirable; this temperature with most mixtures giving me a "dry" mass which absorbs oxygen freely and is readily han- 35

dled. The temperature away from the grinding surfaces may be considerably lower but it is always desirable that the material 40 be hot enough to prevent absorption of much moisture from the air as this would make it pasty and inconvenient to handle.

What I claim is:—

1. The process of making an alkali metal 45 manganate which comprises mechanically comminuting a mixture of manganese oxid and alkali in the presence of air at a temperature sufficient for oxidation.

2. The process of making an alkali metal 50 manganate which comprises comminuting a mixture of manganese oxid and alkali on and with the aid of a hard heated surface in the presence of air, such mixture being at a temperature at which free absorption of 55 oxygen occurs and such surface being at a higher temperature.

3. The process of making an alkali metal 60 manganate which comprises mechanically comminuting a mixture of manganese oxid and alkali in the presence of air and at a temperature around 400° to 550° C.

4. The process of making sodium manganate which comprises mingling fine ground manganese oxid and commercial caustic 65 soda, drying and heating the mixture, and mechanically grinding at a temperature around 400° to 550° C. until a substantial amount of said manganese oxid is converted into sodium manganate. 70

In testimony whereof, I affix my signature hereto.

JOHN R. MacMILLAN.